

Jan. 12, 1943.

R. S. MORSE

2,308,020

DRYING OIL

Filed April 9, 1940

FIG. 1.



FIG. 2.



FIG. 3.



RICHARD S. MORSE  
INVENTOR

BY *Richard S. Morse*  
*Warren K. Cannon*

ATTORNEYS

## UNITED STATES PATENT OFFICE

2,308,020

## DRYING OIL

Richard S. Morse, Rochester, N. Y., assignor to  
Distillation Products, Inc., Rochester, N. Y., a  
corporation of Delaware

Application April 9, 1940, Serial No. 328,702

7 Claims. (Cl. 260—407)

This invention relates to improved procedure for preparing superior bodied or polymerized oils for use in paints, varnishes, inks and the like.

Linseed oil has long been the accepted standard for superior drying oils. However, there has been considerable room for improvement as regards the drying time of linseed oil and the resistance of the linseed oil films to weather resistance, abrasion, etc. Attempts have been made to prepare drying oils from fish oils, but the products have been usually quite unsatisfactory because of tackiness of the film, poor weather resistance, etc.

In Oosterhof Patent 2,065,728, December 29, 1936, and Fawcett 2,128,354, August 30, 1938, it is proposed that bodied vegetable and animal drying oils be improved by subjecting them to high vacuum unobstructed path distillation to remove non-polymerizable materials therefrom. This procedure yields an undistilled residue which has markedly improved characteristics as regards drying time, film hardness, etc.

This invention has for its object to provide a method for preparing improved drying oils satisfactory for paints, varnishes and the like. Another object is to provide improved drying oils. Other objects are to improve the art. Further objects will become apparent from the following description and claims.

These and other objects are accomplished in accordance with my invention which includes subjecting a bodied oil to high vacuum unobstructed path distillation to remove volatiles or non-polymers and then subjecting the undistilled residue to a second bodying treatment. I have discovered that this rebodying of the undistilled residue reduces the drying time to a very short period of time and also increases film hardness, weather resistance and other desirable properties.

The bodied oil which is initially employed in my process, namely, that which is introduced into the still, is preferably bodied by heating to elevated temperature in the substantial absence of oxygen. Catalysts may be employed. This procedure yields a bodied oil of high quality. However, other methods of bodying are well known in the art. Such methods comprise heating while in contact with oxygen, heating while in contact with catalysts. It is also possible to body oils by treatment with ultra-violet light, electric discharge, etc. My invention is applicable to bodied oils produced by any of these known methods.

The bodied oil can be prepared by the bodying of vegetable or marine animal oils which con-

tain polymerizable constituents. At the present time it is commercially unfeasible to polymerize oils having an iodine number below 120 and for this reason I prefer to employ oils having an iodine number of at least 120. This is particularly true in the case of marine animal oils. Examples of oils which may be bodied and used in my invention are linseed, oiticica, soy, walnut, menhaden, sardine, and pilchard oils.

10 The bodied oil is subjected to high vacuum unobstructed path distillation by heating it in a high vacuum and in a still so constructed that the heated oil is separated from the condensing surface by substantially unobstructed space. A pot type unobstructed space still can be employed. However, it is much better to employ a gravity flow type of high vacuum unobstructed path still in which the bodied oil is introduced onto the vaporizing surface and is caused to flow thereover in a thin film by gravity or by forces greater than gravity. Gravity flow type of high vacuum stills are well known in the art and do not require further description. Greater than gravity flow type high vacuum unobstructed path stills are described in Hickman application 99,631. In the preferred form of such stills there is a rotatable vaporizing surface in the form of a disc which is adapted to be heated. A condensing surface is separated therefrom by unobstructed space. During operation the bodied oil is introduced onto the center of the rotating disc and is caused to flow thereover in the form of a very thin film by centrifugal force. During such passage vaporization of non-polymers takes place. I prefer to employ this type of still since it enables rapid distillation without decomposition.

15 The temperatures employed during the distillation will vary considerably depending upon the kind of oil treated and the type of still used. Temperatures of 150–300° C. are best used as far as economic considerations are concerned. Higher or lower temperatures can be used, but with lower temperatures the rate of distillation is uneconomically slow and with higher temperatures decomposition is a problem. Temperatures of about 175° to 275° are preferred. Pressures greater than 2 mm. are usable but are not satisfactory because of increased decomposition.

20 Pressures below about .1 mm. such as .01 to .0001 are best.

25 During the distillation non-polymers and non-polymerizable materials are removed. There are apparently substances in the original oil which inhibit polymerization. These materials are like-

wise removed and this is believed to materially contribute to the value of the subsequent rebodying treatment. The first bodying apparently is incomplete because of the presence of these materials. After their removal rebodying can be carried more nearly to completion yielding a superior product. While proportions involving up to 40% or even more can be removed as distillate, I have found that it is preferable to distill only to remove about 2-12% and particularly about 10%. Little improvement is obtained by removing amounts from 12-30%. A slight improvement takes place between 30 and 40% but I do not regard it as being sufficient to justify removal of more than 12%.

The undistilled residue is then subjected to a bodying treatment. The bodying may be any of the treatments described above in connection with the bodying of the original source material. However, I prefer to employ a bodying treatment which does not involve substantial oxidation and I particularly prefer to employ the conventional bodying treatment involving heating to an elevated temperature while in the presence of an inert gas or while under vacuum. This procedure yields a superior oil of light color.

It is important that the bodying treatment be terminated before the residue is unduly thickened. It is possible to change the undistilled residue into a substance completely unsatisfactory for a paint oil. Apparently the undistilled residue polymerizes quite easily and it is possible for it to be converted into materials which cannot be used satisfactorily in paints and the like. This is particularly true in connection with rebodying by means of oxygen or oxidizing agents. The course of the rebodying can be easily followed by removal of samples and testing and when such tests indicate that the consistency of the oil is that desirable for the particular purpose in mind, the bodying treatment is terminated.

In the accompanying drawing I have graphically illustrated the beneficial results obtained by the procedure of my invention.

Referring to Fig. 1, in which drying time in minutes is plotted against time of rebodying in hours, it is shown that drying time of the undistilled residue is rapidly lessened by rebodying for a period up to about six hours. Thereafter, little advantage is to be obtained by continued bodying. Fig. 1 also shows that the drying time of the undistilled residue can be reduced by approximately 50% by a rebodying time of only one hour. Fig. 1 also illustrates the fact that the undistilled residue from 10% distillate has approximately the same drying time as undistilled residue from 30% distillate and that its characteristics in connection with rebodying are much the same. Therefore, little advantage is to be obtained by removing more than 10 or 12% distillate. However, as remarked above, a slight increase takes place over 30% but does not seem to be sufficient to warrant the added difficulties involved in the distillation.

Fig. 2 illustrates the increase in film hardness by various periods of rebodying in hours in connection with an undistilled residue from a 10% distillate. It is seen that, as far as film hardness is concerned, the effect of rebodying reached a maximum at between two and three hours.

The rebodying treatment in connection with the experiments illustrated in Figs. 1 and 2 involve treating the undistilled residues at 250-270° C. in the presence of nitrogen.

Referring to Fig. 3, it is seen that film hardness is plotted against time of drying or exposure to air in hours. Curve B illustrates the hardness as against time acquired by undistilled residue from a 10% distillate. Curve C shows the film hardness as against time of a residue from a 10% distillate which had been rebodyed for one hour. Curve D shows the film hardness against time for an undistilled residue from a 10% distillate which had been rebodyed for three hours.

#### Example.

Menhaden oil was bodyed by heating in the presence of nitrogen to 250-270° C. for about 15 eight hours. The bodyed product had the following characteristics:

|                          |                  |
|--------------------------|------------------|
| Acid value               | 3.78             |
| Refractive index         | 1.4840 at 40° C. |
| Viscosity-poises         | 10.5 at 25° C.   |
| Iodine value             | 112.0            |
| Percent non-saponifiable | 3.85             |
| Sap. number              | 222.0            |

This bodyed oil was then distilled by passage over a 14 inch centrifugal still plate, heated to a temperature of 180° C. and maintained under a pressure of about .001 mm. 10% of the bodyed oil was removed as distillate. The resulting undistilled residue was tested for drying time by mixing with a commercial drier and spreading on glass in a thin film of .001 mm. thickness which was maintained at room temperature and humidity. Finger smear tests were made every 15 minutes. The undistilled residue had a drying time of 80 minutes as compared with 150 minutes for the original bodyed oil. The undistilled residue was rebodyed by heating in a vacuum for 5 hours at 270° C. It was then mixed with a commercial drier and tested in the same way. It was found that the drying time had been reduced to 20 minutes. The film hardness had been correspondingly improved.

What I claim and desire to be secured by Letters Patent of the United States is:

1. The process which comprises subjecting a bodyed oil to high vacuum unobstructed path distillation in order to remove a member of the group consisting of non-polymers, non-polymerizable materials and polymerization inhibitors and subjecting the undistilled residue to a second bodying treatment which is terminated before the oil loses its valuable paint characteristics.

2. The process which comprises subjecting a bodyed oil to high vacuum unobstructed path distillation in order to remove a member of the group consisting of non-polymers, non-polymerizable materials, and polymerization inhibitors the amount removed being between 2 and 12% of the original oil and then subjecting the undistilled residue to a second bodying treatment which is terminated before the oil loses its valuable paint characteristics.

3. The process of claim 1 in which the second bodying treatment is carried out at elevated temperature for a period of between 1 and 6 hours.

4. The process which comprises subjecting a bodyed oil to high vacuum unobstructed path distillation in order to remove a member of the group consisting of non-polymers, non-polymerizable materials and polymerization inhibitors, and subjecting the undistilled residue to a second bodying treatment which involves heating the residue to an elevated temperature in the sub-

stantial absence of oxygen for a period of about 1-5 hours.

5. The process which comprises subjecting a bodied fish oil having an iodine number above about 120 to high vacuum unobstructed path distillation in order to remove a member of the group consisting of non-polymers, non-polymerizable materials and polymerization inhibitors and then subjecting the undistilled residue to a second bodying treatment which is terminated before the residue loses its valuable paint characteristics.

10 5. The process which comprises subjecting a bodied fish oil having an iodine number of above about 120 to high vacuum unobstructed path distillation in order to remove a member of the group consisting of non-polymers, non-polymerizable materials and polymerization inhibitors and then subjecting the undistilled residue to a second bodying treatment which is terminated before the residue loses its valuable paint characteristics.

15 6. The process which comprises subjecting a bodied fish oil having an iodine number above about 120 to high vacuum unobstructed path distillation in order to remove a member of the group consisting of non-polymers, non-polymerizable

materials and polymerization inhibitors in amounts of not greater than about 10% and subjecting the undistilled residue to a second bodying treatment which is terminated before the residue loses its valuable paint characteristics.

7. The process which comprises subjecting a bodied fish oil having an iodine number of above about 120 to high vacuum unobstructed path distillation in order to remove a member of the group consisting of non-polymers, non-polymerizable materials and polymerization inhibitors in amounts of about 10% and subjecting the undistilled residue to a bodying treatment involving heating to an elevated temperature for a period of less than about six hours.

RICHARD S. MORSE.